# EUROPEAN PATENT SPECIFICATION

(11) **EP 0 090 629 B1**
(45) Date of publication and mention of the grant of the patent: **16.09.1987**
(21) Application number: 83301723.9
(22) Date of filing: 28.03.1983
(51) Int. Cl.: C10M 155/04, C07F 5/04

(54) **Borated lube oil additive**
Borierter Zusatz für Schmieröl
Additif boré pour huile lubrifiante

(30) Priority: 29.03.1982 US 362955
(43) Date of publication of application: 05.10.1983
(73) Proprietor: AMOCO CORPORATION, Chicago Illinois 60601 (US)
(72) Inventor: Anderson, Ronald Leslie, Naperville Illinois 60540 (US)
(74) Representative: Ritter, Stephen David

## Description

This invention relates to a borated reaction product of a long chain aliphatic succinic acid compound and alkylene diamine having an average of at least 2.5 N-substituted hydroxyalkyl groups and lube oil additives containing said borated reaction products.

The patent literature is replete with disclosures of the use of various long chain aliphatic succinic acid compounds in lubricating oil compositions. For example, Lubrizol discloses in U.S. Patents 3,219,666 of Norman et al; 3,381,022 of Le Suer; 3,630,904 of Musser et al; 3,836,471 of Miller; 3,533,945 of Vogel; 3,282,955 of Le Suer; etc. that foreign particles in lubricating oils is a particular problem. U.S. Patent 3,282,955 explains the problem at Column 1, lines 19 to 37 as follows: "One of the principal problems associated with present day automobile crankcase lubricants is that posed by the inevitable presence in the lubricant of foreign particles such as dirt, soot, water, and decomposition products resulting from breakdown of the lubricating oil. Even if there were none of this latter contaminant present the very nature of the design of the modern internal combustion engine is such that a significant amount of foreign matter will accumulate in the crankcase. Perhaps the most important of these contaminants is water because it seems to be responsible for the deposition of a mayonnaise-like sludge. It appears that if there were no water present the solid components of the mayonnaise-like sludge would circulate with the oil and be removed by the oil filter. It will be readily appreciated that the deposition of the sludge presents a serious problem with respect to the efficient operation of the engine and that it is desirable to prevent such deposition of sludge-like material." Subsequently, U.S. Patent 3,630,904 points out at Column 1, lines 42 et seq. that high molecular weight acylated nitrogen compositions have achieved widespread use as ashless dispersants in crankcases and filters. Generally, these ashless dispersants are prepared by reacting high molecular weight mono- or polycarboxylic acid acylating agents with a suitable amine or hydroxy compound. While the patentee indicates that the commercial success of these acylated nitrogen compositions as ashless dispersants is conclusive evidence of their effectiveness as sludge-dispersants, the patentee points out that sludge can and does form on metal surfaces in areas of the engine where water vapor condenses at places such as rocker arms, oil-fill caps, etc.

As indicated above, numerous patents disclose various long chain aliphatic succinic acid derivatives, In somewhat greater detail, U.S. Patents 3,219,666 and 3,640,904 disclose that hydroxyalkyl substituted amines and polyamines can be reacted with long chain aliphatic succinic acid compounds and formulated into lubricating oil compositions. U.S. Patent 3,282,955 discloses the formation of lubricating oil additives based upon borated reaction products of long chain succinic acid compounds and mono-amines, including N-substituted hydroxyalkylated amines. U.S. Patent 3,533,945 discloses lube oil additives based upon borated reaction products of long chain aliphatic succinic acid compounds and polyols. U.S. Patent 3,836,471 discloses lube oil compositions containing the reaction product of long chain aliphatic succinic acid compounds and at least one polyoxyalkylene alcohol demulsifier with the possibility of utilizing amines such as polyalkylene polyamines or hydroxyalkylated polyamines together with the polyoxyalkylene alcohol demulsifier. U.S. Patent 3,630,904 discloses lube oil compositions containing additives formed by reacting adducts of a hydroxyalkylamine and an acylating agent with a long chain aliphatic succinic acid compound. US Patent 4,097,389 of Andress discloses lube oil compositions containing borated oxazoline additives wherein the oxazoline component is a cyclized reaction product of a long chain succinic acid compound and a tris(hydroxymethyl) aminomethane. US Patent 4,071,548 of Okamoto discloses lube oil compositions comprising borated reaction products of long chain aliphatic succinic acid esters and/or amides containing oxyalkylene chains of at least 5 oxyalkylene units. US-A-3,254,025 (Le Suer) discloses a lubricating oil additive prepared by reacting N-hydroxyalkyl substituted alkylene diamine with polyisobutylene-substituted succinic anhydride. The resulting products are borated. However, none of these references discloses borated reaction products of a long chain succinic acid compound and an alkylene diamine having an average of at least 2.5 N-hydroxyalkyl groups and lube oil groups containing these borated reaction products.

While additives prepared from the reaction product of long chain aliphatic succinic acid compounds and alkylene polyamines are excellent lube oil additives, they are inferior to additives where the alkylene polyamine is hydroxyalkylated. In general, the more hydroxyalkyl moieties the greater the dispersancy. However, the products based on hydroxyalkylated polyamines have the drawback that they tend to attack engine seals particularly those of the fluorocarbon polymer type thereby limiting the use of lubricating oils containing these dispersants. Accordingly, there is a need for high dispersancy lube oil additives that do not attack engine seals based on fluorocarbon polymers.

The general object of this invention is to provide a lube oil additive having high dispersancy which is compatible with fluorocarbon engine seals. Other objects appear hereinafter.

We have now found that the objects of this invention can be attained by producing borated reaction products of long chain aliphatic succinic acid compounds and alkylene diamines having on an average at least 2.5 N-hydroxyalkyl groups.

Thus according to the invention there is provided a method of producing a lube oil additive, which comprises the steps of (1) reacting an unsubstituted alkylene diamine with at least 2.5 mols of propylene oxide per mol of alkylene diamine at 50 to 300°C, (2) reacting from 0.5 to 2.0 mols of the resulting N-hydroxyalkyl alkylene diamine with each mol of an alpha long chain aliphatic succinic acid or anhydride at from 0 to 250°C and (3) borating the reaction product of step 2 at 50 to 250°C with sufficient concentration of boron compound to yield a long chain succinic acid product containing at least 0.15% by weight boron.

The additives produced by the method of this invention are particularly well balanced products. While we have found that it is generally desirable to use long chain succinic acid amides and esters based on polyalkylene polyamines having a relatively high concentration of N-hydroxyalkyl moieties because the more N-hydroxyalkyl substituents the cleaner the engine, we have also found that the more amino groups in the polyamine the greater the degradation of fluorocarbon polymer seals. This means that while it is desirable to have a high level of hydroxyalkyl moieties in the additive to enhance engine cleanliness and reduce sludge formation, alkylene amines containing more than 2 amino groups cannot be utilized in this invention. Hydroxyalkylated monoamines do not provide adequate dispersancy. At the same time, it is imperative that the diamine have at least 2.5 N-hydroxyalkyl groups, preferably 2.5 to 4 N-hydroxyalkyl groups, in order to provide acceptable levels of engine cleanliness. Boration is necessary in order to stabilize the additive and reduce engine seal attack. Other things being equal, omission of boration leads to unacceptably high levels of fluorocarbon engine seal attack. However, boration of additives prepared from N-unsubstituted diamines does not reduce fluorocarbon engine seal attack. Accordingly, the lube oil additives of this invention are particularly well balanced.

As indicated the lube oil additives of this invention can be prepared by borating reaction products of an alpha long chain succinic acid compound and an alkylene diamine having on an average at least 2.5 N-hydroxyalkyl groups.

The alkylene diamines useful as starting materials in the method of this invention may have the structure NH₂-R-NH₂ wherein R is an alkylene group of from 2 to 24 carbon atoms, such as ethylene, 1,2-propylene, trimethylene, hexamethylene, dodecamethylene, tetracosene, etc. In general, alkylene diamines containing from about 6 to 12 methylene units are preferred, in order to provide a dispersant having the most advantageous properties, particularly compatibility with the lubricating oil. Hexamethylenediamine is preferred because of its relatively low cost and compatibility of additives prepared from it with lube oils.

As indicated the hydroxyalkylating reactant is propylene oxide. Ethylene oxide is disadvantageous since hydroxyethylated alkylene diamines tend to yield borated dispersants which are slightly incompatible with lubricating oils in the sense that they yield hazy borated products. Ethylene oxide also has the disadvantage that it has a tendency to hydroxyethylate N-hydroxyethylated groups on the diamine thereby reducing the efficiency of the reaction. In contrast propylene oxide yields borated additives which are fully compatible with the lubricating oils and has a reduced tendency to react with N-hydroxypropylated amines. Butylene oxide tends to be less reactive than either ethylene oxide or propylene oxide and is substantially more expensive. The hydroxyalkylating agent can be used in a concentration of about 2 to 6 mols per mol of alkylene diamine. In general approximately 2.5 to 4.5 mols of propylene oxide per mol of diamine is preferred since the final products have about 2.5 to 4 N-hydroxyalkyl groups which provides the best properties at the lowest cost.

The alkylene diamine can be hydroxyalkylated under conventional conditions, i.e. by reaction at 50 to 300°C from 1 to 10 hours.

The long chain aliphatic succinic acid compounds useful in this invention can be prepared by any of the techniques described in the aforesaid patents, which have been incorporated by reference. For example, an acid compound, particularly an ethylenically unsaturated dicarboxylic acid compound (acid or anhydride), such as maleic acid, maleic anhydride, fumaric acid, etc., can be reacted with a suitable olefin or halogenated olefin at a temperature of about 100 to 300°C yielding an alkenyl or alkyl substituted succinic anhydride. If desired the unsaturated groups in the alkenyl group can be removed by standard hydrogenation procedures. Typically, the olefins or halo substituted olefins contain from about 8 to 500 carbon atoms or more and can include homopolymers and copolymers of mono olefins such as ethylene, propylene, 1-butene, isobutene, etc. However, as indicated above any of the techniques utilized in this art can be employed to produce the long chain succinic acid compound.

The long chain aliphatic succinic acid compounds are then reacted with the N-substituted hydroxyalkyl diamine under conditions normally employed in this art at a temperature of from 0 to 250°C. If desired a solvent such as benzene, toluene, naphtha, lube oil, xylene and n-hexane or the like can be used to facilitate the control of the reaction. From about .5 to 2 mols of long chain aliphatic succinic acid compounds can be reacted per mol of N-substituted hydroxyalkyl alkylene diamine. It will be noted that the long chain aliphatic succinic acid compound for purposes of this reaction is difunctional while the N-substituted hydroxy alkylene diamine is tetrafunctional irrespective of the degree of substitution of the alkylene diamine.

The boron compounds useful in this invention include boron oxide, boron dihalides (boron trifluoride, boron tribromide, boron trichloride) boron acids, such as tetraboric acid, metaboric acid and simple esters of the boron acids (trialkyl borates containing 1 to 8 carbon alkyl groups such as methyl, ethyl, n-octyl, 2-ethylhexyl, etc.).

The boron compounds can be reacted with the long chain succinic acid-hydroxy alkylene diamine product at a temperature of from about 50 to 250°C preferably from about 100 to 170°C with a sufficient concentration of boron compound to yield a long chain succinic acid product containing at least .15 percent by weight boron (excluding lube oil). The boron compound can be reacted in a ratio of from 0.1 to 10 moles of boron compound per equivalent of starting long chain succinic acid compound in step 1. This step can be -carried out in the presence of diluent or solvent. In general, the more boron incorporated, the lower the seal attack.

Unless specified in the examples following, percent boron content is always based on lube oil and additive concentration.

### Example I

Four hundred fifteen grams of propylene oxide (7.15 moles) was added dropwise to two hundred sixty-two grams of hexamethylenediamine (2.26 moles) at 150°C in a two liter, 3-necked, round bottom flask fitted with an overhead stirrer, condenser and temperature controller attached to a heating mantle through the top of the condenser over a four hour period while stirring. After the reaction was complete the reaction mass was found to have gained three hundred ninety-five grams (6.81 moles propylene oxide, 95% incorporation) or 3 moles propylene oxide per mole of hexamethylenediamine. The pale yellow N-hydroxypropylated hexamethylenediamine having on an average about 3 hydroxypropyl groups per hexamethylenediamine moiety remained a liquid at room temperature for several days but slowly crystallized to a low melting solid.

One hundred sixty-six grams of the hydroxypropylated hexamethylenediamine (0.571 moles), sixteen hundred grams of a 50% active solution in oil of polybutenyl-succinic anhydride (0.571 moles) having a molecular weight of fourteen hundred, and six hundred forty-nine grams SX-5 base oil were heated at 190°C for two hours in a 3 liter, round bottom, 3-necked flask under a mild nitrogen purge.

The reaction mass was cooled to 130°C and treated with 250 ml xylene and 35.3 grams of boric acid (0.571 moles). The mixture was then refluxed at 140°C with azeotropic removal of water and finally heated to 180°C with a nitrogen purge to remove the xylene. The product (including base oil) was filtered with celite and contained 0.23% boron (0.25% B theoretical) and 0.63 nitrogen (0.66% nitrogen theoretical).

### Example II (Comparative)

This Example illustrates the production of a borated reaction product of a long chain aliphatic succinic acid compound and an unsubstituted alkylene diamine. Twelve hundred grams of a 40.5 percent active solution (in oil) of polybutenyl-succinic anhydride (0.217 moles) having a molecular weight of 2240 and 50.4 grams hexamethylenediamine (0.43 moles) was heated at 100°C for two hours in a 3 liter, 3-necked, round bottom flask. The temperature was then raised to 150°C and nitrogen was blown through the solution to remove excess hexamethylenediamine. The resultant product was treated with ninety-seven grams of boric acid suspended in a Mannich condensation product of polybutylphenol, tetraethylenepentamine and formaldehyde (2.72% boron) overnight at 95°C to yield a product containing 0.20% by weight boron and 0.47% nitrogen.

### Example III (Comparative)

This Example illustrates the production of a borated reaction product of a long chain aliphatic succinic acid compound and alkylene diamine having an average of about 2 N-substituted hydroxypropyl groups. Twenty-four and nine-tenth grams of hydroxypropylated hexamethylenediamine prepared by the method of Example except that a two to one mole ratio of propylene oxide to diamine (0.107 moles) was used, three hundred grams of a 50% active solution (in oil) of polybutenyl-succinic anhydride (0.107 moles) combined with one hundred twelve grams SX-5 base oil were heated at 190°C for two hours in the manner described in Example II. Two hundred grams of this reaction product (0.0490 moles) were treated with 15.2 grams boric acid (0.246 moles) and eight grams of water at 82°C for ninety minutes and then at 170°C for two hours followed by filtration through celite. The final product was shown to be primarily amide and imide by infrared spectroscopy and contained 1.11% B (1.31 theoretical).

### Example IV (Comparative)

This Example illustrates the production of an unborated reaction product of polybutenyl-succinic anhydride and hydroxypropylated hexamethylenediamine having approximately three hydroxypropyl groups per hexamethylenediamine moiety. Sixty-two grams of the hexamethylenediamine propylene oxide reaction product of Example I, twelve hundred grams of a 40% active oil solution of polybutenyl-succinic anhydride having a molecular weight of 2240 (0.214 moles) and ninety-three grams SX-5 base oil were heated at 150°C for five hours with a mild nitrogen purge in a 3 liter, 3-necked flask. The resultant product contained 0.456% nitrogen (0.44 theoretical) and was shown by infrared spectroscopy to be a mixture of ester (1740 cm-¹) and amide (1650 cm-¹).

### Example V

This Example illustrates the preparation of a borated reaction product of polybutenyl-succinic anhydride and hydroxypropylated hexamethylenediamine having approximately three hydroxypropyl groups per hexamethylenediamine moiety and a relatively high boron content. One hundred nineteen grams of the hexamethylenediamine propylene oxide reaction product of Example I, one thousand forty-five grams of a 55% active oil solution of polybutenyl-succinic anhydride having a molecular weight of fourteen hundred (.41 moles) and five hundred seventy-one grams SX-5 base oil were heated at 190°C for two hours with a nitrogen purge in a 5 liter, 3-necked flask. After the reaction mass was cooled to 82°C, one hundred twenty-seven grams boric acid (2.05 moles) and sixty-three grams of water were added. The reaction mixture was slowly heated to 170°C and held at 170°C for two hours and filtered. The final product contained 0.99% boron.

### Example VI

This Example illustrates a comparison of sequence VD engine test of dispersants made according to Examples I, II, IV and V.

The above data shows that a borated unpropoxylated adduct failed the sequence VD test whereas the propoxylated and borated propoxylated adducts of Examples I, IV and V passed the above test. The borated propoxylated adduct of Example V passed the average sludge and piston varnish tests and would pass the average varnish test at a higher concentration.

### Example VII

Dispersants prepared in accordance with the preceding Examples were tested by suspending a fluorocarbon seal in oil solution at 149°C (300°F) for seven days and the change in physical properties (tensile strength percent elongation) was then measured.

The above data clearly shows that boration of an unpropoxylated adduct has no substantial effect upon fluorocarbon seal test results whereas boration of hydroxypropylated dispersants reduces fluorocarbon seal attack as the concentration of boron in the dispersant increases.

### Example VIII (Comparative)

This Example illustrates the production of a borated reaction product of polybutenyl-succinic anhydride and hydroxyethylated hexamethylenediamine having approximately four hydroxyethyl groups per hexamethylenediamine moiety. Three hundred seventy grams hexamethylenediamine (3.19 moles) were heated to 180°C in a one liter, 3-necked round bottom flask fitted with an overhead stirrer fritted glass gas dispersion tube, thermometer and heating mantle. While stirring vigorously, ethylene oxide was added through the gas dispersion tube for six and one-half hours until the product gained five hundred sixty-two grams, corresponding to reaction of 12.77 moles of ethylene oxide (4:1 ratio of ethylene oxide to hexamethylenediamine).

Thirty-five grams of the hydroxyethylated hexamethylenediamine (.120 moles), four hundred fifty grams of a 50% active oil solution of polybutenyl-succinic anhydride (.161 moles) having a molecular weight of 1400, and one hundred sixty-five grams SX-5 base oil were heated at 190°C for two hours with a mild nitrogen purge in the manner described in Example I.

A portion of this product (three hundred eighty-nine grams) was cooled to 100°C and treated with fifty milliliters of xylene and 5.9 grams of boric acid. The mixture was then refluxed at 140°C with azeotropic removal of water and finally heated to 180°C with a nitrogen purge to remove the xylene. The product (including base oil) was filtered with celite and the final product contained 0.11% boron.

## Claims

1. A method of producing a lube oil additive, which comprises the steps of (1) reacting an unsubstituted alkylene diamine with at least 2.5 mols of propylene oxide per mol of alkylene diamine at 50 to 300°C, (2) reacting from 0.5 to 2.0 mols of the resulting N-hydroxyalkyl alkylene diamine with each mol of an alpha long chain aliphatic succinic acid or anhydride at from 0 to 250°C and (3) borating the reaction product of step 2 at 50 to 250°C with sufficient concentration of boron compound to yield a long chain succinic acid product containing at least 0.15% by weight boron.

2. A method according to Claim 1 wherein the propylene oxide is present in a concentration of about 2.5 to 4.5 mols per mol of diamine.

3. A method according to Claim 1 or Claim 2 wherein the alkylene diamine comprises hexamethylenediamine.

4. A method according to any preceding claim wherein the boron compound is reacted in a ratio of 0.1 to 10 mols of boron compound per equivalent of starting long chain succinic acid or anhydride in step 1.

## Patentansprüche

1. Verfahren zur Herstellung eines Schmieröladditivs, dadurch gekennzeichnet, daß man (1) ein unsubstituiertes Alkylendiamin mit wenigstens 2,5 Mol Propylenoxid pro Mol Alkylendiamin bei 50 bis 300°C umsetzt, (2) 0,5 bis 2,0 Mol des erhaltenen N-Hydroxyalkylalkylendiamins mit jeweils 1 Mol einer a-langkettigen aliphatischen Bernsteinsäure oder eines Bernsteinsäureanhydrids bei 0°C bis 250°C umsetzt und (3) das Reaktionsprodukt der Stufe (2) bei 50 bis 250°C mit einer solchen Menge an Borverbindung zur Reaktion bringt, daß sich als Produkt eine langkettige Bernsteinsäure ergibt, die wenigstens 0,15 Gewichtsprozent Bor enthält.

2. Verfahren nach Anspruch 1, dadurch gekennzeichnet, daß das Propylenoxid in einer Konzentration von etwa 2,5 bis 4,5 Mol pro Mol Diamin vorhanden ist.

3. Verfahren nach Anspruch 1 oder 2, dadurch gekennzeichnet, daß das Alkylendiamin Hexamethylendiamin ist.

4. Verfahren nach <«.gendeinem der vorhergehenden Ansprüche, dadurch gekennzeichnet, daß die Borverbindung in einem Verhältnis von 0,1 bis 10 Mol Borverbindung pro Äquivalent an bei der Stufe (1) als Ausgangsmaterial verwendeter langkettiger Bernsteinsäure oder Bernsteinsäureanhydrid umgesetzt wird.

## Revendications

1. Un procédé de production d'un additif pour huile lubrifiante, qui comprend les stades de (1) réaction d'une alcoylènediamine non substituée avec au moins 2,5 moles d'oxyde de propylène par mole d'alcoylènediamine entre 50 et 300°C, (2) réaction de 0,5 à 2,0 moles de la N-hydroxyalcoylalcoylènediamine obtenue avec chaque mole d'un acide ou anhydride succinique à chaîne alpha aliphatique longue, entre 0 et 250°C et (3) boration du produit réactionnel du stade 2 entre 50 et 250°C avec une concentration suffisante d'un composé du bore pour produire un composé d'acide succinique à chaîne longue contenant au moins 0,15% en poids de bore.

2. Un procédé selon la revendication 1 dans lequel l'oxyde de propylène est présent à une concentration d'environ 2,5 à 4,5 moles par mole de diamine.

3. Un procédé selon la revendication 1 ou la revendication 2 dans lequel l'alcoylènediamine comprend l'hexaméthylènediamine.

4. Un procédé selon l'une quelconque des revendications précédentes dans lequel le composé du bore est mis à réagir dans un rapport de 0,1 à 10 moles du composé du bore par équivalent d'acide ou d'anhydride succinique à chaîne longue de départ dans le stade 1.
